# EUROPEAN PATENT APPLICATION

(11) **EP 2 360 286 A1**
(43) Date of publication of application: **24.08.2011**
(21) Application number: 10460002.8
(22) Date of filing: 15.02.2010
(51) Int. Cl.: C23C 2/38

(54) **The method of production a coated wire**

(71) Applicant: Miklasz, Bogumil, 04-848 Warszawa (PL); Dziembaj, Antoni, 05-462 Stefanowka (PL)
(72) Inventor: Miklasz, Bogumil, 04-848 Warszawa (PL); Dziembaj, Antoni, 05-462 Stefanowka (PL)
(74) Representative: Kaczmarczyk, Jan

(57) **Abstract**

The method of production a coated wire consists in introducing a core of the wire (1) into a molted metal and carrying it through a crystallizer (5) in order to produce lagging. During the transition of the core wire (1) through the liquid metal the molecular diffusion of liquid metal atoms into the core of the wire, in plasticity state, takes place and the molecular diffusion of atoms of metal core of the wire (1) into the liquid metal.

## Description

The subject of the invention is the production method of a coated wire having a metal core on which a lag of other metal is placed.

The invention concerns the method of producing the coated wire in a continuous process on an industrial scale.

The materials used for the production the coated wire should have specially chosen features such as a melting temperature and mechanical durability.

The wire being the core of the product should be metallurgically homogenuous, not polluted, and made by a drawing technology.

The soldering method of producing a coated wire has been known. Steel wire being the core of the product is covered with a thin layer of brass and is placed in a covering of cooper sheet. Next, all is heated up to the temperature in which the layers of metals are joined. It is impossible to get a good quality coated wire using this method. Connecting metals by soldering is not long-lasting and, moreover, adding brass interferes with electrical conductivity.

The production of a coated wire in the process of drawing and annealing has been known. Steel wire being the core of the product is lagged with cooper sheet and is subjected to continuous pulling during which a dent in the surface up to the core is obtained and then it is being annealed.

The annealing of a steel wire with a cooper coat takes place in the temperature of about 650 degrees Celsius, which causes the diffusion of cooper atoms into the steel core and iron atoms into cooper. This method requires the selection of materials of specially selected properties. The core wire should be of high purity steel and the coat demands the usage of oxygen-free, vacuum cooper.

Applying this method of producing a coated wire requires high investments and is energy-intensive.

The process is very complicated and requires many operations such as the roughening of the surface of wire, crimping the outer layer of sheet, welding of seam, drawing and annealing.

The electrochemical way of producing a coated wire has been known. This method makes use of the electrolysis and introduces the core wire into the electrolytic bath containing salts of the metal of a coat layer surface.

In the process of electrolysis, under the influence of DC of high intensity, chemically pure metal precipitated from the electrolyte is being deposited on the surface of the core. This way steel or copper wires covered with a layer of silver, copper, chromium, nickel or other metals are being produced.

The production of coated wires with a core of alloy steel or alloys of different metals is also possible. In this method, before the process of electrolysis, the wire passes through the degreasing, washing and electrolytic pickling baths, and after the process it passes through cleaning, finishing touches, and other similar baths.

This method is energy-consuming, requiring large investments and considerable labor. Surfaces of the received coated wires are uneven and porous. Their usage is limited. Electrochemical methods are unfriendly to the environment due to the formation of large quantities of hazardous chemical waste and harmful gas vapors.

The main drawback of the known methods is the ability to perform only thin coating.

The aim of the invention is to develop a new method of producing a coated wire, enabling making the laggings of any thickness assuring high quality and lower manufacturing costs.

The essence in producing a coated wire is putting the wire core into the molten metal, its passage through a crystallizer and exit outside with the wrapping of chilled metal.

Having introduced the core wire into the liquid metal it is being heated to the plasticity temperature.

During the passage of wire through the molten metal a diffusion of liquid metal atoms into the core takes place as well as the diffusion of core atoms into the liquid metal. The method uses metals of different melting temperatures as the core passing through the liquid metal maintains its constant plastic shape.

While passing through a crystallizer the wire is gradually cooled down and the liquid metal of the lagging turns into a solid state. At the outlet of the ctystallizer a wire with a metal lagging permanently connected to the core is obtained.

While manufacturing coated wires of round and regular cross-sections the core wire should be placed into a crystallizer centrally. The core of the wire can not be contaminated.

According to the invention, the method of manufacturing a coated wire enables to produce the wire in a continuous process using industrial methods. In this method there is no restriction as to the thickness of the metal lagging neither to the shape and size, which can be optional, of a cross-section of the finished product. The method, according to the invention is environmentally friendly and meets environmental requirements.

The method of manufacturing a coated wire, according to the invention, is shown in the example of the invention in the device where Figure 1 shows a schematic view of the device and Figure 2 shows a cross-section of the crystallizer. The example demonstrates the way of producing a coated wire with a low carbon steel core with copper lagging.

Steel wire 1 is being placed by the guidance wheel 11, the set of straightening rolls 9 and centering head 4 into the furnace chamber 3 with molten copper of a temperature of 10830 degrees Celsius.

Steel wire 1 heats up from the molten copper to a plasticity temperature of steel and is centrally directed to crystallizer 5 where it is gradually cooled. During the passage of wire 1 through the molten copper the diffusion of copper atoms to the wire 1 and the diffusion of iron atoms to the created copper lagging takes place. In the upper zone 6 and in the central zone 7 of the crystallizer 5 the turning from the liquid copper into the solid state which creates the lagging of the coated wire takes place.

The lower part 8 of the crystallizer 5 is a cooling zone and the coated wire 2 being placed into and having full mechanical strength is pulled outside by a set of pulling wheels 10. In the final phase the coated wire 2 is guided by the directing wheel 12 for being wound on a drum. In the example of the invention the furnace for melting has an atmosphere of nitrogen protecting molten copper from oxidation.

In the method of production, it is important to determine the technological parameters of wire feed rate and cooling of the lower zone of the crystallizer. For wires with a core diameter of 1 mm the speed is about 5 mm / sec.

The method of producing the coated wire, according to the invention, is particularly useful for wires with low-carbon steel or alloy steel core with cooper, aluminum, tin, silver or gold lagging.

High quality coated wires, with a smooth surface are good medium for the surface currents at high frequencies. Such wires can be used for electronic transmission of information, in digital transmission networks type LAN, signaling systems, etc.

Coated wires with steel core which, as a result, has higher mechanical durability can be applied in power industry and rail transport.

## Claims

1. Method of manufacturing the coated wire characteristic by the fact that the core wire (1) is introduced into the molten metal and carried through the crystallizer (5) in order to produce the lagging of a cooling down metal.

2. The method according to claim 1, characteristic by the fact that in the process of transition of the core wire (1) through the liquid metal the molecular diffusion of liquid metal atoms into the wire core (1) in plasticity state takes place and the molecular diffusion of atoms of metal of wire core (1) into the liquid metal.

3. The method according to claim 1, characteristic by the fact that inside the crystallizer (5) a gradual cooling of the wire core (1) takes place, together with the lagging being obtained in a continuous process.

4. The method according to claim 1, characteristic by the fact that the core of the wire (1) in the process of crystallization is set centrally.

## Amended claims

### Amended claims in accordance with Rule 137(2) EPC.

**1.** The method of manufacturing a coated wire characteristic with the fact that the core of the wire (1) is introduced from the top into the centering head (4), having a chamber (13) with a changeable transversal cross-section equipped with centering dividers (14), it is then introduced into the molten metal and conducted through the crystallizer (5) in order to produce the lagging of a cooling down metal.

**2.** The method according to claim 1, wherein the chamber (13) of the centering head (4) has, becoming smaller from the top, a transversal cross-section.

**3.** The method according to claim 1, wherein the centering dividers (14) are separate ones in order to obtain the division of the chamber (13) into the areas with the decreasing volume.

**4.** The method according to claim 3, characteristic with the fact that centering dividers (14) have additional openings to allow the flow of a protective gas through all areas of the chamber (13) between the dividers (14) to ensure the regulation of the temperature rise of the core of the wire (1).

**5.** The method according to claim 1, wherein the position the centering head (4), as to the crystallizer (5), is regulated to ensure the optimal distance of the transition of the core of the wire (1) through the molten metal.
